

June 24, 1930.

R. G. JACKSON

1,765,588

## PROCESS OF MAKING FLOOR COVERINGS

Filed Oct. 13, 1926

2 Sheets-Sheet 1



Inventor

Ralph G. Jackson  
By Cecilia Anne Boyden  
Attorney

June 24, 1930.

R. G. JACKSON

1,765,588

PROCESS OF MAKING FLOOR COVERINGS

Filed Oct. 13, 1926

2 Sheets-Sheet 2



Inventor

Ralph G. Jackson  
Practical Patent Attorney

Attorney

## UNITED STATES PATENT OFFICE

RALPH G. JACKSON, OF WOODBURY, NEW JERSEY

## PROCESS OF MAKING FLOOR COVERINGS

Application filed October 18, 1926. Serial No. 141,396.

This invention relates to floor coverings and has particular reference to a new and improved process of making floor coverings of the felted base type.

In the manufacture of floor coverings employing as a base, a felted material such as asphaltic floor paper, it has been found necessary to seal the base with some material which will prevent the asphalt constituents from seeping through the painted or printed design, especially when a temperature rise is experienced as when drying the painted design by artificial means. It has been proposed heretofore to overcome this difficulty by first coating the material with a lacquer such as a liquid or plastic pyroxylin compound on both sides. The chief objection to this procedure is the expense involved in a process of this character due to the relatively high cost of pyroxylin as compared to paint.

The primary object of the present invention is to provide an improved process for making floor coverings similar to that disclosed in Patent No. 1,562,386, issued November 17, 1925, to C. Marshall Taylor, which shall effectively seal the base in a simple and inexpensive manner and which shall insure a product of high quality and long wearing qualities.

Another object is to provide a novel and improved process consisting of relatively few steps which may be carried out expeditiously and without the use of highly skilled labor.

With these and other objects in view, the invention may be stated to consist in the steps of first coating the felted base material with a relatively quick drying paint, drying the coated base by artificial means then applying thereto a design with a relatively slow drying paint, drying the last mentioned paint by artificial means over a relatively long period, and finally applying a coating of transparent lacquer such as pyroxylin over the design.

In the drawing accompanying and forming part of this application:—

Fig. 1 is a vertical sectional view through

an apparatus for carrying out the first step of my process;

Fig. 2 is a top plan view thereof; and

Figs. 3 and 4 are vertical sectional views through machines illustrating respectively the method of carrying out the second and third steps of my process, namely the application of the design and drying, and applying the transparent lacquer coating and drying.

In carrying out my improved process, I pass the felted base material 1 from a roll 2 through suitable rollers 3 and 3<sup>a</sup>, the latter being adapted to apply a coating of relatively quick drying paint to one side of the material. The paint in this instance may be fed from a supply roller 4 to the roll 3<sup>a</sup>, and thence to one side of the material, and in accordance with this invention I use a paint composed substantially of a pigment, linseed oil, and a low boiling vehicle such as benzine, so that as the material leaves the rolls and passes into a drying room 5 heated by artificial means, the paint may be quickly dried at a temperature well below that which would bring the asphaltic constituents of the base to the surface of the felted material. As an example, the paint used for covering the back of the material may consist of:—500 lbs. talckene, 100 lbs. whiting, 200 lbs. red oxide, 30 gals. oil, 25 gals. naphtha. The above mentioned oil may consist of:—350 lbs. rosin, 17½ lbs. lime, 187 gals. linseed oil, 20 lbs. litharge, 10 lbs. black oxide, 100 gals. varnolene.

The top or wear side of the material may be coated with a paint consisting of:—300 lbs. whiting, 350 lbs. talckene, 30 gals. oil, 5 gals. mixed varnish, 5 gals. varnolene. The oil in the paint for the top side may be the same as used for the bottom side paint. From the above, it will be apparent that the paints applied to both sides of the material have a relatively high content of low boiling point diluent, so that they are of a quick drying nature. The material is illustrated as being supported in festoon arrangement in the drying room in order to expose the painted surface and hasten drying which is accomplished in a relatively short time.

The festoons of material painted on one side are moved slowly through the drying room by suitable conveyors denoted generally at 6, such festoons proceeding along one side of the drying room to a point adjacent the 5 other end whereupon they are turned through 180° and brought back along the opposite side of the drying room as clearly shown in Fig. 2. The material emerging 10 from the drying room is lead back to the paint rollers over suitable angularly disposed guides 7 and 8 so as to present the opposite side of the material to the paint rollers. The material, having been coated 15 on the opposite side, is again dried in the room 5, as above described, and is then rolled up. In this manner I effectively seal the asphaltic constituents in the base in a relatively inexpensive manner, as the aforementioned quick drying paint is easy to apply and comparatively inexpensive to produce.

The roll 10 of material painted on both sides is then fed through a suitable print 25 machine 11 where the desired design units are printed as the base material is moved therethrough with a step by step motion. For this purpose I preferably employ high 30 grade linseed oil paints which dry relatively slowly as compared to the aforementioned 35 base coating and which completely cover the base coating on one side so that a highly durable surface will be presented. As the 40 printed material emerges from the machine 45 11, it is cut into the desired lengths at 12, and is then placed on horizontal racks 13 in an artificially heated drying room 14. The printed material thus placed is subjected to a relatively high temperature over 50 a considerable length of time, as compared to the first mentioned drying room. This 55 procedure thoroughly dries the slow drying painted design and hardens the painted surface so as to present a hard and durable 60 surface.

After the painted design has thoroughly dried and hardened, the strips are removed from the drying room and rolled up to facilitate handling, whereupon each roll 15 is 65 passed between rollers 16 to apply a coating 50 of lacquer over the painted design. These rollers are substantially inflexible lengthwise. They are nine feet long and are eight 55 inches in diameter for the coating of standard width floor coverings of either strip or rug pattern. In practice, I preferably employ a pair of rollers, the upper of which is 60 fitted with a rubber sleeve 17 so that the lacquer coating will be applied evenly to the 65 painted surface, which, due to the design in heavy paints, usually presents an uneven surface. This sleeve is preferably about three-fourths of an inch in thickness and of a density or compactness similar to 70 that of the tread of an automobile tire.

The use of a roller of this character, that is a roller the material of which is softer than the painted floor covering, enables me to apply a substantial coating of lacquer over the entire irregular painted surface which will 75 present a durable wear surface rather than a thin and uneven varnish or finishing surface such as is usually obtained with steel or other non-resilient rollers. It has been found in actual practice that when lacquer is applied by a steel or other non-resilient 80 roller, the raised painted design portions, as contrasted with the background portions, receive a relatively thin or meager lacquer coating, although in use these portions receive the greatest wear. Contrasted to this the present rubber roller and process make it possible to apply sufficient material to such high points so that the lacquer surface 85 can resist the usual wear to which such floor covering is subjected. A resilient roller formed from rubber, as above described, is, of course, non-soluble in the lacquer solvents and hence will last a considerable length of 90 time without appreciable wear or deterioration. The lacquer may be applied from a reservoir 19 located above the rollers and tilted from time to time by hand to flood the upper roller and form a pool on the surface of the material immediately in front 95 thereof as indicated in dotted lines in Figure 4. From the rollers 16, the material passes onto suitable racks 20 which may be horizontal or inclined; as the lacquer dries very quickly and there is little or no danger 100 of its running. Drying is facilitated by enclosing the racks 20 by a suitable enclosure 21 and, if desired, by also passing a heated air draft therethrough.

From the drying enclosure 21, the material 105 is transported to an inspection room where it is marked and packaged.

By the application of lacquer to the painted design surface, it will be obvious that a product of great durability is produced as the lacquer affords a tough coating for the painted design, and after the lacquer wears off the design will withstand considerable wear, due to the use of high grade slow drying paints which completely 110 cover the cheap rapid drying base paint. Since a cheap base paint is employed, a higher grade paint than usual may be employed for the design, together with a lacquer coating thereover, with substantially 115 no increase in cost of the finished product over that of previous processes.

While I have disclosed the first step of my process as applying the sealing coat of paint first to one side of the material, then to the opposite side, it will be obvious that both sides may be coated simultaneously, if desired. Also, the lacquer coating may be applied to both sides of the material after 120 the design has been applied to one side, if 125 130

desired to completely waterproof the entire finished product.

I claim:

1. The process of making floor coverings which consists in the steps of first coating an asphaltic base material on both sides with a quick drying oil paint having a high content of a low boiling diluent and drying said paint by artificial means to quickly seal the asphaltic constituents in the base, and then printing a design on one surface of the painted base with a relatively slow drying paint.

2. The process of making floor coverings which consists in the steps of first coating an asphaltic base material on both sides with an oil paint containing a relatively low boiling point vehicle and quickly drying said paint by artificial means to seal the asphaltic constituents in the base, then printing a design on one surface of the painted base with a relatively slow drying paint, and finally applying a transparent durable coating over the surface containing the design.

3. The process of making floor coverings which consists in the steps of first coating an asphaltic base material on both sides with a quick drying oil paint having a high content of a low boiling diluent and drying said paint by artificial means to quickly seal the asphaltic constituents in the base, then printing a design on one surface of the painted base with a relatively slow drying paint and covering substantially all the quick drying painted surface therewith, and finally applying a transparent pyroxylin coating over the surface containing the design by means of a roller having a resilient surface.

4. The process of making floor covering which consists in the steps of first coating an asphaltic base on both sides with a quick drying oil paint having a high content of a low boiling diluent and drying said paint by artificial means to quickly seal the asphaltic constituents in the base, next printing a design on one surface of the painted base with a slow drying paint and covering substantially all of said surface therewith to provide a durable wearing surface, and finally coating said surface with a transparent pyroxylin compound to render said surface waterproof and further increase the wearing qualities thereof.

5. The process of making floor covering which consists in the steps of first coating an asphaltic base material on both sides with a quick drying oil paint having a high content of a low boiling diluent and drying said paint by artificial means to quickly seal the asphaltic constituents in the base, next printing a design on one surface of the painted base with a slow drying paint and covering substantially all of said surface

therewith to provide a durable wearing surface, then cutting the base thus decorated into predetermined lengths and subjecting such lengths while spread out to artificial drying means, and finally coating each of said lengths with a transparent pyroxylin compound to render said surface waterproof and further increase the wearing qualities thereof.

6. The process of making floor coverings which includes the step of applying a wear coating of a lacquer in substantially even thickness over the irregular contour of a painted design by passing the floor covering between a pair of rollers, and applying a transparent coating solution to the decorated surface by maintaining a pool of the solution on the approach side of the rollers, said rollers engaging said covering sufficiently to draw it therebetween and serving to evenly distribute the solution over the hill and dale surface of the covering in substantially equal thickness over the peaks and depressions, the roller engaging the decorated surface being provided with a surface of yieldable material capable of conforming to the decorated surface whereby any excess of the solution is prevented from collecting in the depressions of the decorated surface.

7. The process of making floor coverings which includes the step of applying a wear coating of a lacquer in substantially even thickness over the irregular contour of a painted design by passing the floor covering with the decorated surface uppermost between two horizontally extending power driven rollers both of a length at least that of the width of the floor covering, and applying a transparent lacquer to the decorated surface by maintaining a pool of the solution on the decorated surface at the approach side of the rollers, said rollers engaging said covering sufficiently firmly to draw it therebetween and serving to evenly distribute the solution over the hill and dale surface of the covering, the roller engaging the decorated surface including an outer yieldably material capable of conforming to the irregularities of the decorated surface whereby excess of the solution is prevented from passing between the rollers and the material is applied with even thickness to both high points and low points on the covering.

In testimony whereof I affix my signature.  
RALPH G. JACKSON.